

## UNITED STATES PATENT OFFICE

2,069,252

## ENAMEL AND VARNISH

Harvey G. Kittredge and Albert J. Turner, Dayton, Ohio, assignors to The Kay and Ess Chemical Corp., Dayton, Ohio, a corporation of Delaware

No Drawing. Application December 28, 1934,  
Serial No. 759,549

4 Claims. (Cl. 134—26)

This invention relates to enamels and varnishes, and particularly to a finish that imitates the appearance of leather, in light colors and pastel shades, which can be baked at a low temperature 5 with the minimum of discoloration. Previously it has been difficult to employ light, delicate colors and pastel shades in baked enamels on account of the discoloration of the varnishes used at the temperature ranges required of from 300 to 400 10 degrees F., and also because of the original dark color of the varnishes employed.

The present invention has the dual purpose of providing an enamel or varnish which dries with an imitation leather finish and which can be 15 pigmented with light, delicate colors that will bake at a temperature of 255 degrees F., and which will not discolor materially so as to change the shades.

It is our object to provide a process of manufacture and a composition of matter which has these qualities. Our invention consists of the manufacture and blending of suitable varnishes and raw China wood oil with or without additional driers, to produce an imitation leather finish in combination with the light colors and pastel shades of 25 the pigments.

## Varnish C

In order to make the first varnish designated as above, we take 100 pounds of Amberol B/S 1 Lt. 30 and 14 gallons of raw China wood oil, heating the China wood oil and the above synthetic resin in a varnish kettle to 550 degrees F. Three pounds of linoleate of lead and one pound of linoleate of cobalt are then added and stirred thoroughly. 35 The batch is then allowed to cool to 450 degrees F. and then reduced with 32 gallons of petroleum naphtha.

Amberol is a phenol, formaldehyde, synthetic resin. It is made as follows: to one hundred parts 40 of phenol aldehyde resin difficultly fusible and only partly soluble in benzol and other solvents and produced, for instance, by heating 108 parts of cresol with 60 to 75 parts of formaldehyde (30% by weight) and distilling off the water and the uncombined cresol, are added gradually to 800 parts of melted colophony. The whole mixture is then heated in an autoclave until a resin is produced which is clear in the cold, homogeneous and free 45 from smell of phenol. The volatile substances are then removed while stirring and 100 parts of glycerol of 28 degrees Bé. are added in small quantities, whereupon the mixture is heated to 250 degrees C. and kept at this temperature for 50 several hours while being stirred carefully. A

typical formula for amberol is shown in United States Patent No. 1,623,901.

## Varnish D

In order to make this varnish we take 200 5 pounds of a pure phenolic resin made by condensing phenol, or a phenol derivative and formaldehyde and twenty gallons of raw China wood oil. We place these in a varnish kettle raising the temperature slowly in about twenty-five minutes to 450 degrees F. We hold at this temperature for twenty minutes. We then thin with 20 gallons of toluol and 60 gallons of petroleum naphtha.

## Example 1

15

A typical varnish or enamel for making a white imitation leather finish is made up as follows:

|                    |       |               |
|--------------------|-------|---------------|
| Varnish C          | ----- | 11½ gallons   |
| Varnish D          | ----- | 6¾ gallons 20 |
| Raw China wood oil | ----- | 1¾ gallons    |

|                                                                  |       |                |
|------------------------------------------------------------------|-------|----------------|
| Thinner composed of equal parts of toluol and petroleum naphtha  | ----- | 1 to 2 gallons |
| Paste composed of pure titanium dioxide ground in a spar varnish | ----- | 120 pounds 25  |

This enamel is applied by spraying. It is then put into an oven at a temperature of 200 to 250 degrees F. and held at approximately 225 degrees for two and a half to three hours. The resulting product will have a wrinkled surface imitating 30 leather. It will appear substantially without discoloration, and provide a smooth, heavy and pebbled surface that is a close imitation of genuine leather.

## Example 2

35

Varnish C and Varnish D can be varied in proportions of two to one of Varnish C to Varnish D, or two to one of Varnish D with respect to Varnish C. Raw China wood oil can be varied in 40 the same combination from one to ten parts. That is, from one to ten gallons, when gallons are used as the measure of the parts. The more China wood oil used, the less the luster, and the finer the finish or grain of the leather.

Different colors may be employed, such as: ultramarine blues; chrome yellows and greens; chromium oxide greens, toluidine and lithol reds, etc.

In the foregoing varnishes the proportions may 50 be varied, but we prefer the proportions indicated, which we have found to be practical varnishes for this purpose.

It will be understood that we desire to comprehend within our invention such modifications as 55

come within the scope of our claims and our invention.

Having thus fully described our invention, what we claim as new and desire to secure by Letters Patent, is:

1. A composition of matter capable of drying in a hard irregular finish upon being baked from 200 to 225 degrees F., comprising a varnish composed of phenolic aldehyde resin 1 part, colophony 8 parts, glycerol 1 part, raw China wood oil, linoleate of lead, linoleate of cobalt and petroleum naphtha; a second varnish composed of a phenolic resin which is a condensate of pure phenol, raw China-wood oil, toluol and petroleum naphtha; raw China wood oil and a thinner of toluol and petroleum naphtha, and a light color paste ground in spar varnish.

2. A composition of matter capable of drying in a hard irregular finish upon being baked from 200 to 225 degrees F., comprising: 100 pounds of a synthetic resin composed of 1 part phenolic aldehyde resin, 8 parts colophony and 1 part glycerol and 14 gallons of raw China wood oil heated to 550 degrees F. with 3 pounds of linoleate of lead and one pound of linoleate of cobalt; cooled to 450 degrees F. and reduced with 32 gallons of petroleum naphtha; a varnish of 200 pounds of pure phenolic condensate resin mixed with 20 gallons of raw China wood oil; heated slowly for approximately 25 minutes to 450 degrees F., and after holding at this temperature for twenty minutes thinned with 20 gallons of toluol and 60 gallons of petroleum naphtha; 1 1/4 gallons of raw China wood oil; one to two gallons of thinner of toluol and petroleum naphtha; and 120 pounds of a light color paste ground in spar varnish.

3. A composition of matter capable of drying in a hard irregular finish upon being baked from 200 to 225 degrees F., comprising: 100 pounds of a synthetic resin composed of 1 part phenolic aldehyde resin, 8 parts colophony and 1 part glycerol and 14 gallons of raw China wood oil heated to 550 degrees F. with 3 pounds of linoleate of lead and one pound of linoleate of cobalt; cooled to 450 degrees F. and reduced with 32 gallons of petroleum naphtha; a varnish of 200 pounds of phenolic resin which is a condensate of pure phenol mixed with 20 gallons of raw China wood oil; heated slowly for approximately 25 minutes to 450 degrees F., and after holding at this temperature for twenty minutes thinned with 20 gallons of toluol and 60 gallons of petroleum naphtha; 1 1/4 gallons of raw China wood oil; one to two gallons of thinner of toluol and petroleum naphtha; and 120 pounds of a light color paste ground in spar varnish.

4. A sprayable enamel for producing imitation leather finishes in light colors comprising 11 1/4 gallons of a varnish composed of 10 lbs. phenol aldehyde resin, 10 lbs. glycerol and 80 lbs. colophony to 3 lbs. linoleate of lead, 1 lb. linoleate of cobalt and 14 gallons of raw China wood oil, mixed with 6 1/4 gallons of a varnish composed of 200 lbs. pure phenol condensate resin to 20 gallons raw China wood oil, 20 gallons toluol and 60 gallons of petroleum naphtha, mixed with 1 to 2 gallons of a thinner composed of equal parts of toluol and petroleum naphtha and combined with 120 lbs. of a paste composed of pure titanium dioxide ground in a spar varnish.

HARVEY G. KITTREDGE. 35  
ALBERT J. TURNER.